

March 11, 1924.

1,486,245

J. H. HASTE ET AL

PHOTOGRAPHIC FILM WITH COLORED LAMINATED BASE

Filed Dec. 26, 1922



INVENTORS  
James H. Haste & Erwin J. Ward,

BY  
R. L. Stinchfield  
ATTORNEY

Patented Mar. 11, 1924.

1,486,245

# UNITED STATES PATENT OFFICE.

JAMES H. HASTE AND ERWIN J. WARD, OF ROCHESTER, NEW YORK, ASSIGNEES TO  
EASTMAN KODAK COMPANY, OF ROCHESTER, NEW YORK, A CORPORATION OF NEW  
YORK.

## PHOTOGRAPHIC FILM WITH COLORED LAMINATED BASE.

Application filed December 26, 1922. Serial No. 609,026.

To all whom it may concern:

Be it known that we, JAMES H. HASTE and ERWIN J. WARD, citizens of the United States of America, residing at Rochester, 5 in the county of Monroe and State of New York, have invented certain new and useful Improvements in Photographic Films with Colored Laminated Bases, of which the following is a full, clear, and exact specification.

This invention relates to photographic films having laminated supports of cellulosic material. The preferred embodiment of the invention relates to colored or pretinted 15 films. The principal object of the invention is to produce such a film in which the coloring material is protected mechanically and chemically by the laminations which make up the support. Other objects will herein- 20 after appear.

In the accompanying drawing the single figure is a diagrammatic sectional view on an exaggerated scale of a film embodying the preferred form of our invention. Where 25 the layers of film blend into each other by a sort of weld continuous outlines are omitted.

Photographic films having a permanent color in the support or base are coming into 30 commercial use in increasing quantities. At present the greatest activity is in the production of motion picture positive films which are pretinted so that the proper tone or effect will be given to the projected picture without the necessity of dyeing the 35 gelatin layer containing the silver image.

Under certain circumstances it is desirable to afford the coloring material greater protection, both mechanically and chemically, 40 than has been done in pretinted films heretofore. We have discovered that such a result may be obtained by locating the coloring material in a relatively thin zone of interunion between two relatively thicker interunited laminations of cellulosic material.

Referring to the drawing, which shows the preferred form of our invention, 1 represents the photographically sensitive layer, say a coating of gelatino-silver-haloid emulsion. The support for the emulsion comprises two supporting layers 2 which are preferably composed of compositions of cellulosic addition compounds, such as nitrocellulose, cellulose acetate and cellulose ether.

The compositions may, of course, contain the 55 usual modifying agents, such as high boiling solvents or softeners, as will be readily understood by those skilled in the art.

The layers 2 are joined together by a cement or solvent in such a way as to cause a 60 relatively thin layer or zone 3 of interunion. The entire adjacent faces of the layers 2 are thus blended together, so as to form a practically inseparable support. The coloring material is applied in or by means of 65 the cement or solvent which effects the interunion and thus the coloring material is located in the zone 3, where it is protected from all of the developing, fixing, washing and, above all, bleaching baths to which the 70 film may be subjected. It is likewise located away from the rear surface of the film which is sometimes subjected to scratching when motion picture positive film is run through apparatus of defective design 75 or defective condition.

The layers 2 are preferably flexible and transparent, and it is desirable, in the preferred form of our invention, that the colored zone of interunion 3 be likewise 80 transparent. The cement is selected with this end in view. Any good transparent film cement containing a suitable coloring material, such as a spirit dye, for instance, may be employed. Also a solvent mixture 85 for softening the surfaces of the layers 2 before pressing them together may be employed instead of a cement containing a cellulosic material. Here again a spirit dye can be employed. By way of example, we 90 note the following useful composition for effecting the union,—acetone 20 parts, methyl alcohol 20 parts, methyl acetate 40 parts, butyl acetate 19 parts, and nitrocellulose a trace, say 1 part. To this may be added a 95 spirit dye, the amount of dye depending upon the depth of color desired. Safranine is an instance of one of the dyes that can be used.

The zone 3 may contain just enough color 100 of the right shade to neutralize any objectionable color in the layers 2. This is indicated in our prior application, Serial No. 594,562, filed Oct. 14, 1922 for photographic film with base of neutral tint, the present 105 application being a continuation in part thereof.

Having thus described our invention, what

we claim as new and desire to secure by Letters Patent is:

As an article of manufacture, a pretinted photographic film comprising a photographically sensitive layer, and a flexible light-transmitting laminated support therefor which includes two relatively thick transparent layers of cellulosic addition compound interunited throughout their adja-

cent faces, the relatively thin zone of inter-<sup>10</sup>  
union being colored and being protected  
mechanically and chemically by said thick  
layers.

Signed at Rochester, New York, this 20th  
day of Dec., 1922.

JAMES H. HASTE.  
ERWIN J. WARD.